

J. OLIVER.  
Casting Mold-Boards.

No. 147,157.

Patented Feb. 3, 1874.

Fig. 1.



Fig. 2.



WITNESSES:

P. C. Dietrich  
Harry G. Scott

INVENTOR

James Oliver

per: C. H. Watson & Co.  
ATTORNEYS.

# UNITED STATES PATENT OFFICE.

JAMES OLIVER, OF SOUTH BEND, INDIANA.

## IMPROVEMENT IN CASTING MOLD-BOARDS.

Specification forming part of Letters Patent No. 147,157, dated February 3, 1874; application filed January 14, 1874.

### CASE B.

*To all whom it may concern:*

Be it known that I, JAMES OLIVER, of South Bend, in the county of St. Joseph and State of Indiana, have invented certain new and useful Improvements in Casting Plow Mold-Boards; and I do hereby declare that the following is a full, clear, and exact description thereof, reference being had to the accompanying drawings and to the letters of reference marked thereon, which form a part of this specification.

My invention relates to the process of casting beveled bolt-holes in mold-boards when cast on chills; and the nature of my invention consists in providing the chill with holes for the reception of wooden or metal pins; also, in cores provided with central holes, and in pins, made either of wood or metal, to pass through the cores into the holes in the chills, as will be hereinafter more fully set forth.

In order to enable others skilled in the art to which my invention appertains to use the same, I will now proceed to describe how my process is carried out, referring to the annexed drawing, in which—

Figure 1 is a plan view of the drag of the mold, with the chill and pattern in place; and Fig. 2 is a transverse vertical section through the line  $x x$ , Fig. 1.

A represents the drag, and B the cope, of the mold or flask. C is the chill, and D the

pattern. Into the face of the chill C are drilled very fine holes  $a$ , about one-eighth of an inch deep, where the bolt-holes are wanted in the mold-board. Into these holes I place close-fitting pins  $d$ , made either of wood or metal. On that part of the pin that projects above the face of the chill, I place a beveled metallic core,  $b$ , having a hole through its center of the same size as the holes in the face of the chill. When the pins  $d$  are made of wood, the melted iron, of which the mold-boards are made, destroys them, and the cores remain in the holes of the casting without damaging them or injuring the chill during the operation of contraction. When using metal pins, they are made of wire, and the contraction of the casting in cooling removes them from the holes in the chill without damage to the chill or casting.

Having thus fully described my invention, what I claim, and desire to secure by Letters Patent, is—

The beveled perforated core  $b$ , perforated chill C, and pin  $d$ , when constructed and arranged as and for the purpose set forth.

In testimony that I claim the foregoing as my own I affix my signature in presence of two witnesses.

JAMES OLIVER.

Witnesses:

R. C. THOMPSON,  
F. C. NIPPOLD.